

Aug. 15, 1944.

M. A. FERST ET AL

2,355,639

PENCIL LEAD

Filed May 19, 1943

*Fig. 1.*



*Fig. 2.*



*Fig. 3.*



Inventors

Monie A. Ferst and  
Charles F. Wysong

By *Jewett and Ward*  
Attorneys

## UNITED STATES PATENT OFFICE

2,355,639

## PENCIL LEAD

Monie A. Ferst and Charles F. Wysong, Atlanta,  
Ga., assignors to M. A. Ferst, Ltd., Atlanta, Ga.,  
a corporation of Georgia

Application May 19, 1943, Serial No. 487,654

17 Claims. (Cl. 120—83)

The invention relates to pencil leads or marking elements of ceramic character and has as an object the provision of an element of increased strength against breaking, as compared with existing elements of a comparable grade of softness or hardness.

It is a further object of the invention to provide a marking element which will have improved uniformity of character in all parts of each individual element, as well as among the individual elements in each grade of softness or hardness.

It is a further object of the invention to provide a marking element which will carry a larger proportion of the impregnant material than comparable elements now in use.

In the drawing accompanying and forming a part hereof

Figure 1 is a side elevation of a pencil lead somewhat enlarged.

Figure 2 is a detail vertical section very greatly enlarged of the material of Figure 1, and

Figure 3 is a similar cross sectional view.

In the drawing no attempt has been made to show the different elements in their correct proportions nor to show correct relative sizes of the materials. As shown enlarged impregnated pores are indicated at 10, graphite masses or particles at 11 and the bond material at 12. For purpose of illustration the pores or lacunae 10, which are formed as described below, are shown very much exaggerated in size as compared with the graphite particles 11 and the presumably plate-like bond portions 12.

The dimensions of the particles of graphite are measurable in microns and the particles of material used to form the pores 10 are also exceedingly minute, therefore the showing of the drawing is idealized and a correct showing of relative sizes or proportions is impossible, particularly where a wide variation is possible with the invention.

By "porosity" is meant the percentage of pores by volume of the specimen ready for impregnation which can be filled by gas or liquid. The range of porosity of graphitic lead pencil leads now in use is between sixteen per cent for hard leads and forty per cent at the outside for soft leads. In accordance with the present invention the percentage of porosity is increased by an amount sufficient to have an appreciable effect on the character of the finished element. An increase of as little as five per cent is sufficient to secure some of the advantages of the invention.

Graphitic marking elements such as are in common use in lead pencils are ceramic in character and are preponderantly composed of powdered graphite as a marking material and finely divided clay as a bond which bond is glassy in character as a result of the firing step of manufacture. The finest particles of the clay are as small as substantially one-tenth micron and may range to substantially two microns while the graphite particles usually range between about one micron and a possible eighty microns in well made elements.

The naturally occurring interstices between particles of such sizes are exceedingly small. Furthermore it is considered desirable in the art, to so choose the different sizes of particles of the material as to provide as compact a body as possible for resultant strength and uniformity, but with resultant reduction of capacity for impregnant.

In accordance with the present invention, an increase in porosity is brought about by inclusion of material in the mix, while preparing the same for molding, which added material is affected or removed during the process of manufacture to leave an additional volume of pores in the body of the completed marking element. The material so included may be removed by volatilization, by extraction with a solvent, or the added material may be reduced in volume as by charring.

The ideal result contemplated by the present invention may be obtained by a choice of graphite and bond particle sizes such as to result in no porosity, that is maximum compactness, and a provision of removable material, or material whose volume could be reduced by treatment, in quantity and in fineness of particle size to provide the exact size and number of pores desired for a particular result.

The porosity would then be under full control and if the mixing is properly done, the result would be maximum uniformity. It is desirable to approach as closely as possible to this ideal.

Among the materials that may be charred or otherwise reduced in volume in the firing of the lead are soaps, vegetable dusts or fibers and synthetic fibers. Such substances while not completely removed are sufficiently reduced in volume to provide increased porosity in predetermined amount.

Examples of materials that may be removed prior to or during the firing step are naphthalene, waxes, sulphur and other organic materials.

A separate class of substances which may be used for the purpose of the invention is finely divided metal or metallic salts reducible to free metal under firing conditions. The resulting metal in the fired lead can then be removed by the use of a weak acid or base. A usable metal for this purpose is copper or its salts. The noble metals are also usable where expense will permit.

After the lead has been otherwise completed with the increased porosity desired, it is impregnated. The impregnant can and is understood to include any and all liquids and/or solvents and/or all solids which can be converted into liquids by solvents or heat.

A result of the practice of the process of the invention is that the new leads so produced have the bonded graphitic mass interspersed with impregnant filled pores or lacunae of substantially increased size whereby the marking material yields more readily to abrasion and is consequently more friable for a given flexural or point strength. If an oil and/or a waxy impregnant is used the increased proportion of oil and/or wax provides greater lubrication resulting in a smoother mark. The function of the oil and/or wax impregnant being to cause the graphite to adhere to the paper, the mark will appear more intense. Further, the porosity being controlled, the leads of the invention will have a more uniform body and, also, be more uniform in marking and in writing in every degree of softness and hardness.

A number of different impregnants are contemplated in the impregnation of the porous body of the invention. The impregnant may contain water soluble coloring matter in which case the lead will produce a graphite mark or a colored graphite mark and if the color is water soluble to sufficient extent a copying pencil lead will be provided of the so-called indelible type. The impregnant may be a water soluble chromate in which case the lead will produce a mark that can be used for transfer purposes. The impregnant, which is water soluble can contain an ionogen in which case the lead will produce a mark which will conduct electricity. The conductivity can be controlled by the amount of ionogen used.

It is important that the material of the lead aside from the porosity producing material shall be as compact as possible to provide a strong skeleton interspersed with the pores produced by the removed material.

A pencil lead made in accordance with the invention will be stronger for a comparable softness and softer for a comparable strength than the usual pencils since the impregnant adds strength to the material.

The increase in breaking strength is not inconsistent with an increase of yield to abrasion noted above. The element may be regarded as a skeleton of graphite and bond surrounding the impregnant filled pores. As wear exposes a pore the surrounding skeletal substance will present edges thereof backed up—as resisting abrasion—only by the impregnant which of itself has little resistance to displacement. Therefore, the abrasion can break off some of the skeletal material and rub off some of the impregnant into adherence to the paper. In resistance to flexure, however, the impregnant filled pores are interspersed with the skeletal material and can only yield by flow of the material since it is substantially incompressible.

A pencil lead made in accordance with the invention will be more uniform in marking and

in writing in any given degree of softness or hardness because porosity will be more accurately controlled. The writing qualities of a lead are drastically altered by any change in porosity, other factors being equal. The pores normally developed in formation are subject to much variation due to variations in water content, extrusion pressure, method of tempering and so forth. The type of pores developed by this invention will be unaffected by most of these factors, hence they would be more uniform than the normal pores. Since the two types of porosity would be additive, the overall uniformity would be improved.

10 The expression "reduced in volume" as used in the appended claims includes the reduction to zero or complete removal of the distending material.

15 Minor changes may be made in the steps of the process or in the characteristics of the article produced thereby within the scope of the appended claims, without departing from the spirit of the invention.

We claim:

20 1. The process of producing graphitic marking elements which comprises: preparing a mixture including graphite, bonding material, and a discrete distending material; forming a marking element thereof; firing the thus formed element; subjecting the element, at some stage subsequent to the forming operation, to treatment acting to reduce the volume of the distending particles, and filling the thus formed pores with an impregnant.

25 2. The process of producing graphitic marking elements which comprises: preparing a mixture comprising graphite, clay, and a discrete distending material; forming a marking element thereof; firing the thus prepared element; subjecting the material, at some stage subsequent to the forming operation, to treatment to remove the particles of distending material so as to leave vacant the spaces occupied thereby during formation of the element; and filling said vacant spaces with an impregnant.

30 3. The process of producing graphitic marking elements which comprises: preparing a mixture comprising graphite, bonding material and a discrete vaporizable distending material; said last named material comprising from five to forty per cent by volume of the mass; forming a marking element from the thus prepared mix, firing the formed element with consequent vaporization of the distending material; and filling the resulting pores with an impregnant.

35 4. The process of claim 3 wherein the distending material is powdered naphthalene.

40 5. A graphitic marking element comprising a body formed of graphite and bonding material and having pores throughout the mass, the total volume of the pores being abnormally large, said pores filled with an impregnant.

45 6. A graphitic marking element comprising a skeletal body of graphite particles bonded together by fired clay, enclosing pores which are of a larger volume than the volume of the interstices normally occurring between particles of graphite and bond of marking elements, said pores filled with impregnant.

70 7. The structure of claim 5 wherein the impregnant is an oily and/or waxy material.

8. The structure of claim 5 wherein the impregnant is an oily and/or waxy material containing oil or wax soluble materials.

9. The structure of claim 5 wherein the im-

pregnant is an oily and/or waxy material containing a wax soluble coloring material.

10. The structure of claim 5 wherein the impregnant is a water soluble waxy material.

11. The structure of claim 5 wherein the impregnant is a water soluble waxy material containing a water soluble coloring material.

12. The structure of claim 5 wherein the impregnant is a water soluble chromate.

13. The structure of claim 5 wherein the impregnant is water soluble.

14. The structure of claim 5 wherein the impregnant is a water soluble containing ionogen.

15. The structure of claim 5 wherein the impregnant is a hydroscopic and water soluble material containing ionogen.

16. The structure of claim 6 wherein the excess volume is at least five per cent.

17. The process of producing graphitic marking elements which comprises: preparing a mixture including finely divided graphite and bonding material, the sizes and quantities of each size of particles of the material chosen to provide a minimum of voids, adding at least five per cent by volume of discrete material to said mixture; forming a marking element of said mixture; firing the thus formed element; subjecting the element, at some stage subsequent to the forming operation, to treatment acting to reduce the volume of the particles of the discrete material; and filling the thus formed pores with an impregnant.

MONIE A. FERST.  
CHARLES F. WYSONG.